

## UNITED STATES PATENT OFFICE

2,126,504

## SENSITIZED BLUE PRINT PAPER AND COATING THEREFOR

Alger P. Reynolds, North Beverly, Mass., assignor to Spaulding-Moss Company, Boston, Mass., a corporation of Massachusetts

No Drawing. Application August 21, 1937.  
Serial No. 160,309

## 1 Claim. (Cl. 95—7)

The present invention relates to the art of making "blue prints" by coating a suitable base (which base for the sake of convenience is hereinafter referred to as "paper", but which expression is intended to cover any suitable base which may be used, such as paper, cloth, etc.) with a solution which is sensitive to light so that when the sensitized paper is subsequently exposed to light and then subjected to a suitable developing bath a permanent blue color is obtained wherever the light reached the sensitized paper during exposure.

The primary object of my invention is to provide a more highly sensitive coating for blue print paper which requires exposure to light a shorter period of time during printing, thereby providing a faster paper.

Another object is to provide such a coating which results in a deeper blue background in the exposed areas in the final print.

A further object is to eliminate fogging of the white unexposed surfaces or lines in the final print.

Another object is to provide such an improved sensitized paper which may be kept for longer periods of time in sensitized condition without deterioration prior to exposure to light.

A further object is to provide a coating solution which may be applied to the paper at room temperature, i. e., without heating the solution during coating.

Other objects are to provide an improved blue print paper coating and an improved coating solution.

In the prior art it has long been the established practice to sensitize the paper with a coating solution having as its essential elements a water solution of a light-sensitive iron salt in the ferric state, such as ferric ammonium oxalate, and a suitable ferricyanide, such as potassium ferricyanide. When the coated paper has been dried it is fully sensitized and ready for use and is known commercially as "blue print" paper.

In use, an opaque diagram upon transparent or translucent paper (or other suitable medium) is transposed over the sensitized surface of the blue print paper and is then exposed to light for a period of time sufficient to insure reduction of the light-sensitive ferric salt to a ferrous salt. Upon washing the exposed paper with water the ferrous salt combines with the ferricyanide to form an insoluble blue compound, and the unexposed and un-reduced ferric salt which is found on the blue print paper beneath the opaque lines of the dia-

gram is dissolved out of the blue print paper leaving a white diagram upon a blue background. After being washed with water the exposed paper is commonly washed in a bath containing an oxidizing agent, such as potassium bichromate, thereby bringing out in full the blue background and the paper is then again washed with water and subsequently dried.

Either partial or complete substitution of a ferrocyanide for the ferricyanide in the above-referred to prior art coating bath has been suggested to thereby obtain a faster printing paper which gives sharper white lines upon a deeper blue background. These suggestions will be found in the British patent to Holden No. 418,369 of 15 1934. In the only suggestions of the use of ferrocyanide found in the prior art, it has been stated that the entire coating solution, i. e., water, light-sensitive ferric salt and ferrocyanide (and ferricyanide, if the latter is also used) must not 20 be acid, and this coating solution as a whole has been made either neutral or alkaline by the use in the solution of suitable combinations of borax, ammonia, sodium hydroxide or potassium oxalate, and the use of these chemicals has been understood by the art to be "buffering" the coating solution to neutral or above, i. e., neutral or alkaline.

When an alkali metal ferrocyanide, such as potassium, sodium or ammonium ferrocyanide, is added to a water solution of a light-sensitive ferric salt, such as ferric ammonium oxalate, an insoluble blue substance is formed before exposure to light and after exposure and washing a paper coated with such a coating solution retains a considerable amount of the blue substance upon the unexposed areas, so that these unexposed areas are fogged with blue rather than remaining a clear white. Thus if a ferrocyanide is to be used in a coating solution something must be present which prevents the retention of this blue substance upon the unexposed areas thus permitting it to be washed completely off after printing, leaving clear whites. The prior art has believed that the incorporation of any suitable "buffer" in this ferrocyanide coating solution to thereby make the solution as a whole neutral or alkaline would prevent this fogging of the whites.

In my copending application Serial No. 65,661, filed February 25, 1936, I have pointed out that when one or more of the class comprising alkaline hydrolyzable alkali metal compounds are used in a ferrocyanide coating in such proportions that the water solution of the coating is acid, a greatly improved paper results in that fogging of the

whites is eliminated, the paper prints faster, with sharper white lines upon a deeper blue background and the coated paper is easier to keep in sensitized condition.

5 The group of chemicals known as the alkali metal phosphates includes some phosphates which are acid hydrolyzable in a water solution and some phosphates which are alkaline hydrolyzable in a water solution. I have discovered 10 that the acid hydrolyzable alkali metal phosphates may be incorporated in a coating solution containing a light-sensitive iron salt in the ferric state, and an alkali metal ferrocyanide to give as improved, if not a better coating than is obtained by the use of alkaline hydrolyzable 15 alkali metal compounds or alkaline hydrolyzable alkali metal phosphates. I do not know why the acid hydrolyzable alkali metal phosphates are as satisfactory for this purpose as the alkaline hydrolyzable alkali metal compounds, but so far as I know they are the only acid hydrolyzable substances which function per se in the coating to prevent the formation of an insoluble blue compound prior to exposure to light. Thus the alkali metal phosphates as a class are particularly 20 adaptable for use in such a ferrocyanide blue print coating since both those which are acid hydrolyzable and those which are alkaline hydrolyzable are fully operative to produce the desired result.

By the term "alkali metal" in this specification and the annexed claim, I intend to include only potassium, sodium, cesium, rubidium, lithium, and ammonia, which latter substance although it is not, strictly speaking, a metal, is commonly classed in the alkali metal group. By "alkaline hydrolyzable" compounds wherever said term is used in this specification and the annexed claim, I intend to include only water soluble salts or compounds, the water solutions of which have a pH value of greater than 7. By "acid hydrolyzable" compounds wherever said term is used in this specification and the annexed claim, I intend to include only water soluble salts or compounds, the water solutions of which have a pH value of less than 7.

Thus the class of chemicals referred to as "alkali metal phosphates" includes such chemicals as:

- 50 a. Monosodium phosphate, monopotassium phosphate and monoammonium phosphate.
- b. Sodium pyrophosphate, trisodium phosphate and disodium phosphate.
- c. Sodium borophosphate, sodium glycerophosphate, ammonium sodium phosphate and magnesium ammonium phosphate.

The examples set forth in paragraph a are "acid hydrolyzable alkali metal phosphates", i. e. each hydrolyzes acid in a water solution and the examples set forth in paragraphs b and c are "alkaline hydrolyzable alkali metal phosphates". The examples set forth in paragraph c are so-called "complex" alkali metal phosphates, i. e. alkali metal phosphates in which one or more alkali metals and one or more phosphate radicals are present. I intend to include such complex alkali metal phosphates within the term "alkali metal phosphates" even if such phosphates contain in addition metals other than alkali metals or acid radicals other than phosphate radicals.

Other members of the alkali metal phosphate class will be apparent to persons skilled in the art.

75 An example of a coating solution using an acid

hydrolyzable alkali metal phosphate is as follows:

6000 grams ferric sodium oxalate and 5 552 grams monopotassium phosphate dissolved in 15,000 cc. of water, and to this solution add:

422 grams potassium ferrocyanide and 10 329 grams potassium ferricyanide dissolved in 15,000 cc. of water.

This solution is of a deep blue color and has a pH value of 3.97. If the ferricyanide is replaced in whole or in part by ferrocyanide the amount of monopotassium phosphate should ordinarily be increased.

15 Examples of coating solutions using alkaline hydrolyzable alkali metal phosphates are as follows:

6000 grams ferric ammonium oxalate and 20 900 grams sodium pyrophosphate, dissolved in 15,000 cc. of water, and to this add:

900 grams potassium ferrocyanide and 15 750 grams potassium ferricyanide dissolved in 15,000 cc. of water.

This solution is of a deep blue color and has a 25 pH value of 6.19.

6000 grams ferric sodium oxalate and 30 2485 grams sodium glycerophosphate dissolved in 15,000 cc. of water, and to this add:

422 grams of potassium ferrocyanide and 35 329 grams of potassium ferricyanide dissolved in 15,000 cc. of water.

This solution is of a deep blue color and has a 40 pH value of 6.02.

If the ferricyanide is replaced in whole or in part by ferrocyanide in either of the foregoing solutions the respective amounts of sodium pyrophosphate and sodium glycerophosphate should 45 ordinarily be increased.

It will be apparent to one skilled in the art that if alkali metal ions are present in a coating solution containing a light-sensitive ferric salt and a ferrocyanide, the incorporation of phosphates or any phosphoric acid into such a solution to thereby form an alkali metal phosphate would be within the scope of this invention as equivalent to use ab initio of an alkali metal phosphate.

It will be apparent to persons skilled in this art 50 that it is within the scope of this invention and the annexed claim to first coat the paper with a solution containing, or to prepare a paper with a sizing containing, one or more alkali metal phosphates and then to subsequently coat this paper with a solution containing a light-sensitive ferric salt and a ferrocyanide, since the two coatings would combine to form the coating of this invention.

In this specification and the annexed claim 55 when I refer to a coating containing alkali metal phosphates, light-sensitive iron salts in the ferric state, and ferrocyanides, I intend to include a coating solution containing, a coating containing, and a paper coated with a coating containing the reaction products of said alkali metal phosphates, said light-sensitive ferric salts and said ferrocyanides because I do not know whether or not said chemicals retain their original identity after 60 they are brought together in a coating solution or a coating.

It will be understood that the use of ferrocyanide may be entirely eliminated in any of my coating solutions hereinabove described, and also 65

70 75

that the proportions of ferricyanide to ferrocyanide may be varied at will as has been indicated. Generally speaking the more ferricyanide present in relation to the ferrocyanide present, 5 the slower is the printing speed.

It will also be understood that more than one of the alkali metal phosphates may be used in the same coating solution even though these compounds are selected from different subclasses as 10 defined in this specification.

It will be further understood that chemicals other than alkali metal phosphates, light-sensitive ferric salts, ferrocyanides, and ferricyanides may be incorporated in the coating solution or in 15 the coating on the paper without departing from my invention. So long as the water solution of the coating is acid and contains at least one alkali metal phosphate, a light-sensitive ferric salt, and an alkali metal ferrocyanide, it is intended to be 20 within the scope of the annexed claim, even if the coating solution or the coating on the paper contains other chemicals in addition to those specified.

Suitable light-sensitive iron salts in the ferric 25 state other than ferric ammonium or ferric sodium oxalate, suitable alkali metal ferrocyanides other than potassium ferrocyanide, and suitable ferricyanides other than potassium ferricyanide will be apparent to those skilled in the 30 art.

The determination of the alkalinity, neutrality, or acidity of hydrolyzation of the compounds and salts recited in this specification and the determination of the pH values of coating solutions given 35 in this specification has been made by utilizing a potentiometer and a glass electrode, which method is well known to those skilled in the art. By an acid coating solution I mean one which has a pH value of less than 7 and which value is determined 40 by said method or by one which is equivalently accurate. By an alkaline hydrolyzable compound or salt I mean one the water solution of which has a pH value greater than 7 and which value is accurately determined by said method or its 45 equivalent. By an acid hydrolyzable compound or salt I mean one the water solution of which has a pH value of less than 7 and which value is accurately determined by said method or its equivalent.

In use the paper is sensitized by coating at 50 least one surface thereof with a coating solution made in accordance with this invention, and it is then dried and ready for use. Such a coated paper is dark blue-green in color as distinguished from the lemon-yellow color of prior art paper. 55 The coating may be effected by brushing, by spraying, by passing the paper through a machine

in contact with rollers which dip into a bath of the solution or by any other suitable coating procedure. The diagram is then superimposed upon the sensitized surface of the dry paper, is printed by exposure to light, and the printed or exposed 5 paper is passed through a water bath after which it may be hung up to dry. If desired, before this final drying the paper may be passed through an oxidizing bath, then through another water bath and then dried. 10

The acidity of the coating solution as a whole increases the speed of reduction of the light-sensitive iron salt and thus an acid coating solution provides a much faster printing paper than a coating solution which is neutral or alkaline. 15

Paper coated with the acid coating solutions of a light sensitive ferric salt and ferrocyanide made in accordance with my invention may be kept in sensitized condition without spoilage for much longer periods of time before exposure than the 20 papers of the prior art, and will produce perfectly clear and unfogged whites when subsequently printed. The acidity of my coating solution causes the size in the paper to swell and thus to absorb the coating solution much more readily 25 than neutral or alkaline solutions, and consequently a less concentrated coating solution is required to provide sufficient of the sensitized coating upon the surface of the paper for a satisfactory deep blue background in the final print, 30 whereas in the use of neutral or alkaline solutions it is necessary to use solutions which are highly concentrated and which require heating to keep the chemicals in solution before and during 35 coating.

It is to be understood that my invention is not dependent upon the theories which I have set forth as descriptive of the chemical actions involved nor dependent upon the soundness or accuracy of theoretical statements so advanced, 40 such theories or theoretical statements are merely what I believe to be correct and I intend to claim everything inherent in my invention which is novel in view of the prior art. 45

I claim:

A sensitized blue print paper coating containing an acid hydrolyzable alkali metal phosphate, a light-sensitive iron salt in the ferric state and an alkali metal ferrocyanide, the proportions of said alkali metal phosphate to the other ingredients of the coating being such that a water solution of said coating has a pH value of less than 7 but not sufficiently low to permit the formation 50 of an insoluble blue compound prior to exposure to light.

ALGER P. REYNOLDS. 55